



US005411855A

**United States Patent** [19]

MacIntyre et al.

[11] **Patent Number:** **5,411,855**[45] **Date of Patent:** **May 2, 1995**[54] **PHOTOGRAPHIC ELEMENT EXHIBITING  
IMPROVED SPEED AND STABILITY**

[75] Inventors: Gladys L. MacIntyre, Clyde; Roger Lok, Rochester, both of N.Y.

[73] Assignee: **Eastman Kodak Company**,  
Rochester, N.Y.[21] Appl. No.: **168,834**[22] Filed: **Dec. 16, 1993**[51] **Int. Cl.<sup>6</sup>** ..... G03C 1/34; G03C 1/005[52] **U.S. Cl.** ..... 430/603; 430/604;  
430/611; 430/567; 430/569[58] **Field of Search** ..... 430/603, 604, 611, 567,  
430/569[56] **References Cited****U.S. PATENT DOCUMENTS**

|           |        |                  |       |         |
|-----------|--------|------------------|-------|---------|
| 2,394,198 | 2/1946 | Mueller          | ..... | 95/7    |
| 3,361,564 | 1/1968 | Bigelow et al.   | ..... | 96/64   |
| 3,445,235 | 5/1969 | Burt             | ..... | 96/95   |
| 3,451,819 | 6/1969 | Haugh            | ..... | 96/95   |
| 3,607,288 | 9/1971 | Burt             | ..... | 96/101  |
| 3,647,455 | 3/1972 | Burt et al.      | ..... | 96/64   |
| 3,655,390 | 4/1972 | Overman          | ..... | 96/108  |
| 3,656,952 | 4/1972 | Miller           | ..... | 96/48   |
| 3,782,959 | 1/1974 | Bigelow          | ..... | 96/107  |
| 4,150,993 | 4/1979 | Suga et al.      | ..... | 96/64   |
| 4,835,093 | 5/1989 | Janusonis et al. | ..... | 430/567 |
| 4,933,272 | 6/1990 | McDugle et al.   | ..... | 430/567 |
| 5,079,138 | 1/1992 | Takada           | ..... | 430/567 |

**FOREIGN PATENT DOCUMENTS**

|         |         |                    |   |
|---------|---------|--------------------|---|
| 0325235 | 7/1989  | European Pat. Off. | . |
| 0348934 | 1/1990  | European Pat. Off. | . |
| 0368304 | 5/1990  | European Pat. Off. | . |
| 0369424 | 5/1990  | European Pat. Off. | . |
| 0369491 | 5/1990  | European Pat. Off. | . |
| 0371338 | 6/1990  | European Pat. Off. | . |
| 0435355 | 7/1991  | European Pat. Off. | . |
| 0457298 | 11/1991 | European Pat. Off. | . |
| 1572125 | 8/1975  | Germany            | . |
| 1572140 | 8/1975  | Germany            | . |
| 3908835 | 3/1989  | Germany            | . |
| 1105235 | 3/1988  | Japan              | . |
| 3237453 | 2/1990  | Japan              | . |
| 3208041 | 8/1994  | Japan              | . |

**OTHER PUBLICATIONS**

Wiss. Photolab. Publication, Translation 63(1965), pp. 63-72.

*Primary Examiner*—Thorl Chea  
*Attorney, Agent, or Firm*—Peter C. Cody[57] **ABSTRACT**

The present invention provides a photographic element comprising a support having thereon a silver halide emulsion layer. The emulsion layer contains an organic compound having a thiosulfonic acid substituent, an organic compound having a sulfinic acid substituent, and an amine borane.

**20 Claims, No Drawings**

## PHOTOGRAPHIC ELEMENT EXHIBITING IMPROVED SPEED AND STABILITY

### FIELD OF THE INVENTION

This invention relates to photographic elements. In particular, it relates to novel photographic silver halide elements exhibiting high sensitivity and excellent resistance to storage changes.

### BACKGROUND OF THE INVENTION

For more than a century, it has been known that certain materials are sensitive to actinic radiation and, upon exposure to such radiation, form latent images capable of being subsequently developed into a useful visible image. Almost exclusively, commercial application of these radiation sensitive materials has been the domain of silver halides which exhibit superior sensitivity to light over other radiation sensitive materials, some of which have been known for as long as silver halides have been in use. Such superior sensitivity has made silver halides more practical for use in cameras and other photographic equipment since they can be utilized in low light situations, or in situations where the mechanical characteristics of a camera (or other exposure means) would interfere with an optimum exposure.

Because it is desirable to improve the sensitivity of silver halide crystals, and hence the photographic elements in which they are contained, photographic chemists have over the years attempted to vary the processes for making, or the components within, silver halide emulsions. Typically, the process of making photographic emulsions has consisted of the following steps:

1. The formation of a dispersion of microcrystals (grains) of silver halide in a solution of protective colloid.
2. Physical ripening to achieve the desired grain size.
3. The freeing of the dispersion from excess soluble salts by washing or by coagulation followed by redispersal in a salt free medium.
4. A heat treatment, often in the presence of sensitizing agents, to increase light sensitivity. The treatment is variously termed after-ripening, second ripening, chemical ripening, or digestion.
5. Addition of agents that confer the desired properties, such as sensitizing dyes, antifoggants and stabilizers, and hardeners.

It is during these steps that photographic chemists have added additional components to the emulsion, or varied the conditions under which the emulsion is formed, in order to optimize certain emulsion characteristics. One such characteristic is contrast, and it is generally desired that contrast be maximized.

High contrast is desirable because it is directly related to the appearance of sharpness in an emulsion. One measure of contrast is the sharpness of the toe section of an emulsion's D-log E curve. By sharpness of the toe section, it is usually meant the relative density of the toe section. For instance, a sharp toe corresponds to a relatively low (small) toe density, and a soft toe corresponds to a relatively high (large) toe density. Generally, the point at which toe density is measured corresponds to 0.3 log E fast of the speed point, which is defined as the point on the D-log E curve where density equals 1.0.

It has been known that improvements in the contrast of photographic emulsions can be obtained by employing various transition metals as either dopants or grain

surface modifiers. Dopants are substances added to an emulsion during silver halide precipitation which typically become incorporated within the internal structure of the silver halide grains. Grain surface modifiers, by contrast, are added post-precipitation, thus becoming associated with the surface of the silver halide grains rather than their internal structure.

Recently, emulsion dopants have been described which comprise transition metal complexes having nitrosyl or thionitrosyl ligands. European Patent Applications 0325235 and 0457298 disclose the use of one such complex, namely potassium ferric pentacyanonitrosyl. A second type of dopant, rhenium nitrosyl or rhenium thionitrosyl is disclosed in U.S. Pat. No. 4,835,093; and a third, dicesium pentachloronitrosyl osmate, is disclosed in U.S. Pat. No. 4,933,272. The third is known, in certain instances, to increase the contrast of photographic emulsions. It does so, however, at the expense of a corresponding decrease in sensitivity. Sensitivity (or "speed") of an emulsion is usually defined as the reciprocal of the relative amount of light in Log E  $\times 100$  to produce 1.0 density.

It has been recognized in the art that photographic sensitivity can be increased by adjusting the pH and/or the pAg of a silver halide emulsion. It has also been known that enhanced photographic sensitivity can be obtained by the addition of certain types of chemical sensitizers. Several types of sensitizers have been identified. The most prevalent are gold and sulfur compounds, both of which are thought to enhance emulsion speed by forming electron or photohole traps on the silver halide crystal surface.

Sensitization has also been accomplished by the addition of other transition metals. Specifically, platinum salts have been used, although sensitization with such salts is strongly retarded by gelatin. In addition, iridium salts and complex ions of rhodium, osmium, and ruthenium have been used as chemical sensitizers. The overall effect of these metals on sensitivity appears to be dependant upon their valence state.

Reduction sensitization is another means by which sensitivity enhancement can be obtained. Known reducing agents include stannous chloride, ascorbic acid (as in European Patent Applications 0369491 and 0369424) and dimethylamine borane (U.S. Pat. Nos. 4,150,093 and 3,782,959). However, the use of such sensitizers, as well as other types of sensitizers described above, often causes an indiscriminant, and undesirable, reduction of silver ions to silver atoms. The silver atoms give rise during development to a generally or locally developed density that is not associated with the action of the image forming exposure. This density is typically termed fog and it is best measured as the minimum density on the emulsion's D-Log E curve ( $D_{min}$ ).

Fog is undesirable because it is an indication that the discrimination between the photographic image and the unexposed area is reduced. Thus, the quality of the image obtained is less than optimal. For silver chloride emulsions, which are more prone to being reduced than emulsions containing silver bromide or silver iodide (or mixtures thereof), this problem is even more severe.

A problem closely linked with fog is the tendency for silver halide emulsions, whether chemically sensitized or not, to exhibit unwanted sensitometric changes—such as an increase in speed—during their storage (aging). The ability of an emulsion to be resistant to

these storage changes is called the emulsion's stability (or "keeping ability").

To improve an emulsion's stability, and to control the formation of fog, it has been known to add to the emulsion chemicals known as antifoggants and stabilizers. Because some of these compounds function in both capacities often only one compound is added.

Known antifoggants include the mercaptotetrazoles, tetraazaindenes, benzothiazolium salts, and the thiosulfonates. The thiosulfonates, in particular, have been the subject of much study in recent years. Examples of their uses can be found in the following references: European Patent Applications 0369424, 0435355, 0371338, 10 0368304, 0348934, U.S. Pat. No. 5,079,138, German Patent 3,908,835, JO3,237,453 and JP4,083,241, as well as in S. Gahler in Veroff. wiss. Photolab. Wolfen X, 15 63(1965), and in Z. Wiss. Photo. 63 133(1969).

Thiosulfonates, and especially their alkali salts, suffer the disadvantage of being particularly prone to decomposition. Such decomposition, if not carefully controlled, often gives rise to unacceptable photographic emulsions exhibiting variable speed and high fog.

One method of improving the antifoggant/stabilizer effects of thiosulfonates is to incorporate them into an emulsion along with an amount of sulfinate salt. U.S. Pat. No. 2,394,198 discloses an improvement in the effects of sulfinate salts by the addition to silver halide emulsions amounts of thiosulfonates. Japanese Kokai 3-208041 discloses the use of thiosulfonates and sulfonates during grain formation to make the antifogging effect more obvious. European Patent Application 0358170 discloses the use of thiosulfonates and sulfonates in a direct positive emulsion.

Although the combination of thiosulfonates and sulfonates is known, emulsions containing this combination lack the desired degree of sensitivity and resistance to storage changes. It is therefore desired to provide photographic emulsions which contain thiosulfonates and sulfonates, and which exhibit high sensitivity and resistance to storage changes. Furthermore, it is desired that such emulsions exhibit their characteristics without exhibiting any significant loss in contrast.

#### SUMMARY OF THE INVENTION

The present invention provides a photographic element comprising a support having thereon a silver halide emulsion layer, wherein the emulsion layer contains an organic compound having a thiosulfonic acid substituent, an organic compound having a sulfonic acid substituent, and an amine borane.

The combination of these compounds in a silver halide emulsion, and especially an emulsion which is predominantly silver chloride, imparts to the emulsion the advantageous characteristics of high sensitivity and excellent resistance to storage changes. When the above compounds are used in an emulsion together with a transition metal complex comprising a nitrosyl or thionitrosyl ligand and a transition metal selected from groups V to X, inclusive, of the periodic table, the advantages of the invention are realized without any significant loss of contrast in the emulsion.

The present invention also provides for a method of improving the sensitivity and stability of a silver halide emulsion. Such method comprises adding to the emulsion an organic compound having a thiosulfonic acid substituent, an organic compound having a sulfonic acid substituent, and an amine borane. In a preferred em-

bodiment, the method also comprises the step of adding a transition metal complex to the emulsion.

#### DETAILED DESCRIPTION OF THE INVENTION

The present invention concerns silver halide elements which contain several adjuvants and which exhibit the desired characteristics of high sensitivity and stability. Specifically, the elements contemplated by the present invention contain a combination of antifoggant/stabilizer compounds. The first of these is an organic compound having a thiosulfonic acid substituent; the second is an organic compound having a sulfonic acid substituent. They are structurally defined below by formulas I and II, respectively:



For each compound the R substituent, whether R<sup>1</sup> or R<sup>2</sup>, independently represents an aliphatic, carbocyclic (which includes an aryl), or heterocyclic group, which may be substituted or unsubstituted. Preferably, the R substituents are independently selected from the group consisting of an unsubstituted or substituted alkyl of 1 to 22 carbon atoms, an unsubstituted or substituted aryl group having 6 to 20 carbon atoms, or an unsubstituted or substituted 3-membered to 15-membered heterocyclic group having one or more heteroatoms.

Examples of suitable aliphatic groups include methyl, ethyl, propyl, butyl, pentyl, hexyl, octyl, ethylhexyl, decyl, dodecyl, hexadecyl, octadecyl, isopropyl, t-butyl, butenyl, propargyl, and butynyl.

Examples of suitable carbocyclic groups are phenyl, tolyl, naphthyl, cycloheptatrienyl, cyclohexyl, cyclooctatrienyl, and cyclononatrienyl.

Examples of suitable heterocyclic groups are pyrrole, furan, tetrahydrofuran, pyridine, picoline, piperidine, morpholine, pyrrolidine, thiophene, oxazole, thiazole, imidazole, selenazole, tellurazole, triazole, tetrazole, and oxadiazole.

Groups suitable for substitution on R<sup>1</sup> or R<sup>2</sup> include alkyl groups (for example, methyl, ethyl, hexyl), fluoroalkyl groups (for example, trifluoromethyl), alkoxy groups (for example, methoxy, ethoxy, octyloxy), aryl groups (for example, phenyl, naphthyl, tolyl), hydroxy groups, halogen groups, aryloxy groups (for example, phenoxy), alkylthio groups (for example, methylthio, butylthio), arylthio groups (for example, phenylthio), acyl groups (for example, acetyl, propionyl, butyryl, valeryl), sulfonyl groups (for example, methylsulfonyl, phenylsulfonyl), acylamino groups, sulfonylamino groups, acyloxy groups (for example, acetoxy, benzoxy), carboxy groups, cyano groups, sulfo groups, and amino groups.

The R substituents may further be associated with one or more divalent linking groups. The linking groups include an atom or group containing at least one atom of carbon, nitrogen, sulfur, or oxygen. Examples include alkylene, alkenylene, alkynylene, arylene, O, S, NH, CO, and SO<sub>2</sub>. When such a linking group is present in the antifoggant/stabilizer compound, the compound is a polymer, with its repeating unit being the compound defined by formula I or II and the divalent linking group.

For each of the compounds represented by formulas I and II, M<sup>1</sup> and M<sup>2</sup> independently represent any mono-,

di-, or tri-valent cation. Thus,  $M^1$  and  $M^2$  include metal ions such as sodium ions, potassium ions, calcium ions, and lithium ions, as well as, ammonium ions and phosphonium ions. Preferably,  $M^1$  and  $M^2$  represent sodium ions.

In a preferred embodiment of the present invention, the emulsions contain an organic compound having a thiosulfonic acid substituent (formula I) in an amount between about 10 and about 2300 milligrams per mole of silver halide, and an organic compound having a sulfinic acid substituent (formula II) in an amount between about 10 and about 20,000 milligrams per mole of silver halide, with the ratio of the compound containing the thiosulfonic acid substituent to the compound containing the sulfinic acid substituent being between about 20:1 and about 1:20 by weight. Preferably, the emulsions contain an organic compound having a thiosulfonic acid substituent in an amount between about 100 and about 1500 milligrams per mole of silver halide, and an organic compound having a sulfinic acid substituent in an amount between about 100 and 15,000 milligrams per mole of silver halide, with the ratio of thiosulfonic acid substituent to sulfinic acid substituent being between about 10:1 and about 1:10 by weight.

Optimally, the above-described compounds are tolyl-thiosulfonate salts and tolylsulfinate salts, respectively. They, and other preferred examples of antifoggants/stabilizers, can be synthesized by methods known in the art and described, for example, in *Journal of Organic Chemistry*, vol. 53, p. 386 (1988) and *Chemical Abstracts*, vol. 59, 977e.

In accordance with the present invention, the contemplated elements also contain an amine borane, which may be generically defined by the following structural formula:



wherein  $R^3$ ,  $R^4$ , and  $R^5$  represent hydrogen atoms, aliphatic, carbocyclic (including aryl), or heterocyclic groups, which may be substituted or unsubstituted. Optimally,  $R^3$  is an alkyl or hydroxyalkyl group having 1 to 20 carbon atoms; and  $R^4$  and  $R^5$  are alkyl or hydroxyalkyl groups each having 1 to 20 carbon atoms, or hydrogen atoms.

Examples of suitable aliphatic groups include methyl, ethyl, propyl, butyl, pentyl, hexyl, octyl, ethylhexyl, decyl, dodecyl, hexadecyl, octadecyl, isopropyl, t-butyl, butenyl, propargyl, and butynyl.

Examples of suitable carbocyclic groups are phenyl, tolyl, naphthyl, cycloheptatrienyl, cyclohexyl, cyclooctatrienyl, and cyclononatrienyl.

Examples of suitable heterocyclic groups are pyrrole, furan, tetrahydrofuran, pyridine, picoline, piperidine, morpholine, pyrrolidine, thiophene, oxazole, thiazole, imidazole, selenazole, tellurazole, triazole, tetrazole, and oxadiazole.

Substituents suitable for substitution on  $R^3$ ,  $R^4$ , and  $R^5$  include those disclosed for  $R^1$  and  $R^2$ .

Specific amine boranes suitable for the invention are exemplified by trimethylamine borane, tertiary butylamine borane, dimethyl dodecylamine borane, ethanolamine, diethanolamine, pyridine borane, and picoline borane. The amine boranes are preferably incorporated into the emulsion in amounts between about 0.001 and about 1.0 milligram per mole of silver halide. A more preferred level of incorporated amine borane is between about 0.02 and about 0.2 milligrams per mole of silver halide. Ideally, the amine borane of the present invention is dimethylamine borane and it is incorporated into the emulsion in an amount equal to about 0.05 to about 0.1 milligram per mole of silver halide.

The amine borane reduction sensitizer, as well as the compounds of formulas I and II, may be added to a black and white or color emulsion at any time during the preparation of the photographic element. It is preferred, though, that they be added post-precipitation and just prior to coating the emulsion on a support.

It is also preferred that the above compounds be added to emulsions comprised of predominantly silver chloride. Although it is specifically contemplated that the advantages of the invention would be present in emulsions containing silver halide grains of any known type (silver bromide, chloride, or iodide, or mixtures thereof) or form (i.e. cubic, octahedral, dodecahedral, spherical or tabular), silver chloride content of at least 70 molar percent and silver iodide content of less than 2 molar percent is preferred. Even more preferred is an emulsion containing 98 molar percent silver chloride, with the remaining silver halide being silver bromide and silver iodide. Most preferred is an emulsion containing silver chloride as the sole silver halide.

Irrespective of the type of grains employed in the present invention, it is preferred in certain embodiments of the invention that such grains be internally or externally modified by a dopant or grain surface modifier. Utilization of modified grains enables the emulsion to exhibit the desired characteristics of high sensitivity and excellent stability without also exhibiting the loss of contrast which is often observed in emulsions containing reduction sensitizers.

The dopant or grain surface modifier suitable for the invention is preferably a transition metal complex. It may be generically defined by the formula:



where

$M$  is a transition metal selected from the Groups V to X, inclusive, of the periodic table adopted by the American Chemical Society and published in the *Chemical and Engineering News*, Feb. 4, 1985, p.26;

$Z$  is oxygen or sulfur, and together with nitrogen forms the nitrosyl or thionitrosyl ligand;

$L$  represents a ligand additional to the nitrosyl or thionitrosyl ligand;

$m$  is from 4 to 7, preferably 5 or 6; and

$n$  is zero, -1, -2, or -3.

The ligands defined above by  $L$  can represent virtually any known type of ligand. Any combination of ligands is contemplated. Specific examples of preferred ligands include aquo ligands, halide ligands, cyanide ligands, cyanate ligands, thiocyanate ligands, selenocyanate ligands, tellurocyanate ligands, azide ligands, and other nitrosyl or thionitrosyl ligands.

Preferred dopants and grain surface modifiers include:

|       |                          |
|-------|--------------------------|
| TMC-1 | $[V(NO)(CN)_5]^{-3}$     |
| TMC-2 | $[Cr(NO)(CN)_5]^{-3}$    |
| TMC-3 | $[Mn(NO)(CN)_5]^{-3}$    |
| TMC-4 | $[Fe(NO)(CN)_5]^{-2}$    |
| TMC-5 | $[Ru(NO)Cl_5]^{-2}$      |
| TMC-6 | $[Ru(NO)Br_5]^{-2}$      |
| TMC-7 | $[Ru(NO)I_5]^{-2}$       |
| TMC-8 | $[Ru(NO)F_5]^{-2}$       |
| TMC-9 | $[Ru(NO)Cl_3(H_2O)_2]^0$ |

-continued

|        |                                                              |
|--------|--------------------------------------------------------------|
| TMC-10 | $[\text{Ru}(\text{NO})\text{Cl}_3(\text{H}_2\text{O})]^{-1}$ |
| TMC-11 | $[\text{Ru}(\text{NO})\text{Cl}_4(\text{OCN})]^{-2}$         |
| TMC-12 | $[\text{Ru}(\text{NO})\text{Cl}_4(\text{CN})]^{-2}$          |
| TMC-13 | $[\text{Ru}(\text{NO})\text{I}_4(\text{TeCN})]^{-2}$         |
| TMC-14 | $[\text{Ru}(\text{NO})\text{Cl}_4(\text{SCN})]^{-2}$         |
| TMC-15 | $[\text{Ru}(\text{NO})\text{Br}_4(\text{SeCN})]^{-2}$        |
| TMC-16 | $[\text{Ru}(\text{NO})\text{I}_4(\text{SeCN})]^{-2}$         |
| TMC-17 | $[\text{Ru}(\text{NO})\text{Cl}_3(\text{CN})_2]^{-2}$        |
| TMC-18 | $[\text{Ru}(\text{NO})\text{Br}_2(\text{CN})_3]^{-2}$        |
| TMC-19 | $[\text{Ru}(\text{NO})\text{I}_2(\text{CN})_3]^{-2}$         |
| TMC-20 | $[\text{Ru}(\text{NO})\text{Cl}_4(\text{N})_3]^{-2}$         |
| TMC-21 | $[\text{Ru}(\text{NO})\text{Cl}(\text{CN})_4]^{-2}$          |
| TMC-22 | $[\text{Ru}(\text{NO})\text{Br}(\text{SCN})_4]^{-2}$         |
| TMC-23 | $[\text{Ru}(\text{NO})\text{(SCN})_4]^{-2}$                  |
| TMC-24 | $[\text{Ru}(\text{NO})\text{I}(\text{CN})_5]^{-2}$           |
| TMC-25 | $[\text{Os}(\text{NO})\text{Cl}_5]^{-2}$                     |
| TMC-26 | $[\text{Os}(\text{NO})\text{Br}_5]^{-2}$                     |
| TMC-27 | $[\text{Os}(\text{NO})\text{I}_5]^{-2}$                      |
| TMC-28 | $[\text{Os}(\text{NO})\text{F}_5]^{-2}$                      |
| TMC-29 | $[\text{Os}(\text{NO})\text{Cl}_4(\text{TeCN})]^{-2}$        |
| TMC-30 | $[\text{Os}(\text{NO})\text{Br}_4(\text{OCN})]^{-2}$         |
| TMC-31 | $[\text{Os}(\text{NO})\text{I}_4(\text{TeCN})]^{-2}$         |
| TMC-32 | $[\text{Os}(\text{NO})\text{Cl}_4(\text{SeCN})]^{-2}$        |
| TMC-33 | $[\text{Os}(\text{NO})\text{Br}_4(\text{SeCN})]^{-2}$        |
| TMC-34 | $[\text{Os}(\text{NO})\text{I}_4(\text{SeCN})]^{-2}$         |
| TMC-35 | $[\text{Os}(\text{NO})\text{Cl}_3(\text{CN})_2]^{-2}$        |
| TMC-36 | $[\text{Os}(\text{NO})\text{Br}_2(\text{CN})_3]^{-2}$        |
| TMC-37 | $[\text{Os}(\text{NO})\text{I}_2(\text{SCN})_3]^{-2}$        |
| TMC-38 | $[\text{Os}(\text{NO})\text{Cl}_2(\text{SCN})_3]^{-2}$       |
| TMC-39 | $[\text{Os}(\text{NO})\text{Cl}(\text{CN})_4]^{-2}$          |
| TMC-40 | $[\text{Os}(\text{NO})\text{Br}(\text{CN})_4]^{-2}$          |
| TMC-41 | $[\text{Os}(\text{NO})\text{(SCN})_4]^{-2}$                  |
| TMC-42 | $[\text{Os}(\text{NO})\text{(CN})_5]^{-2}$                   |
| TMC-43 | $[\text{Re}(\text{NO})\text{Cl}(\text{CN})_5]^{-2}$          |
| TMC-44 | $[\text{Re}(\text{NO})\text{Cl}_5]^{-2}$                     |
| TMC-45 | $[\text{Re}(\text{NO})\text{Br}_5]^{-2}$                     |
| TMC-46 | $[\text{Re}(\text{NO})\text{Cl}_2(\text{CN})_3]^{-2}$        |
| TMC-47 | $[\text{Ir}(\text{NO})\text{Cl}_5]^{-1}$                     |
| TMC-48 | $[\text{Ir}(\text{NO})\text{Br}_5]^{-1}$                     |
| TMC-49 | $[\text{Ir}(\text{NO})\text{I}_5]^{-1}$                      |
| TMC-50 | $[\text{Ir}(\text{NO})\text{Cl}_3\text{Br}_1]^{-1}$          |
| TMC-51 | $[\text{Ru}(\text{NS})\text{Cl}_5]^{-2}$                     |
| TMC-52 | $[\text{Os}(\text{NS})\text{Br}_5]^{-2}$                     |
| TMC-53 | $[\text{Ru}(\text{NS})\text{I}_5]^{-2}$                      |
| TMC-54 | $[\text{Os}(\text{NS})\text{Cl}_4(\text{N}_3)]^{-2}$         |
| TMC-55 | $[\text{Ru}(\text{NS})\text{Br}_4(\text{N}_3)]^{-2}$         |
| TMC-56 | $[\text{Os}(\text{NS})\text{I}_4(\text{N}_3)]^{-2}$          |
| TMC-57 | $[\text{Ru}(\text{NS})\text{Cl}_4(\text{CN})]^{-2}$          |
| TMC-58 | $[\text{Os}(\text{NS})\text{Br}_4(\text{CN})]^{-2}$          |
| TMC-59 | $[\text{Ru}(\text{NS})\text{I}_4(\text{CN})]^{-2}$           |
| TMC-60 | $[\text{Os}(\text{NS})\text{Cl}_4(\text{SCN})]^{-2}$         |
| TMC-61 | $[\text{Ru}(\text{NS})\text{Br}_4(\text{SCN})]^{-2}$         |
| TMC-62 | $[\text{Os}(\text{NS})\text{I}_4(\text{SCN})]^{-2}$          |
| TMC-63 | $[\text{Ru}(\text{NS})\text{Cl}_4(\text{SeCN})]^{-2}$        |
| TMC-64 | $[\text{Os}(\text{NS})\text{Br}_4(\text{SeCN})]^{-2}$        |
| TMC-65 | $[\text{Ru}(\text{NS})\text{I}_4(\text{SeCN})]^{-2}$         |
| TMC-66 | $[\text{Os}(\text{NS})\text{Cl}_3(\text{N}_3)_2]^{-2}$       |
| TMC-67 | $[\text{Ru}(\text{NS})\text{Br}_3(\text{CN})_2]^{-2}$        |
| TMC-68 | $[\text{Os}(\text{NS})\text{Cl}_3(\text{SCN})_2]^{-2}$       |
| TMC-69 | $[\text{Ru}(\text{NS})\text{Cl}_2(\text{SeCN})_2]^{-2}$      |
| TMC-70 | $[\text{Ru}(\text{NS})\text{Cl}_2(\text{N}_3)_3]^{-2}$       |
| TMC-71 | $[\text{Os}(\text{NS})\text{I}_2(\text{CN})_3]^{-2}$         |
| TMC-72 | $[\text{Os}(\text{NS})\text{Br}_2(\text{SCN})_3]^{-2}$       |
| TMC-73 | $[\text{Ru}(\text{NS})\text{Cl}_2(\text{SeCN})_3]^{-2}$      |
| TMC-74 | $[\text{Ru}(\text{NS})\text{Cl}_2(\text{N}_3)_3]^{-2}$       |
| TMC-75 | $[\text{Os}(\text{NS})\text{I}_2(\text{CN})_3]^{-2}$         |
| TMC-76 | $[\text{Ru}(\text{NS})\text{Br}_2(\text{SCN})_3]^{-2}$       |
| TMC-77 | $[\text{Os}(\text{NS})\text{Cl}_2(\text{SeCN})_3]^{-2}$      |
| TMC-78 | $[\text{Os}(\text{NS})\text{Cl}(\text{N}_3)_4]^{-2}$         |
| TMC-79 | $[\text{Ru}(\text{NS})\text{I}(\text{CN})_4]^{-2}$           |
| TMC-80 | $[\text{Ru}(\text{NS})\text{Cl}(\text{SCN})_4]^{-2}$         |
| TMC-81 | $[\text{Os}(\text{NS})\text{Cl}(\text{SeCN})_4]^{-2}$        |
| TMC-82 | $[\text{Ru}(\text{NS})\text{(CN})_5]^{-2}$                   |
| TMC-83 | $[\text{Ru}(\text{NS})\text{(SCN})_5]^{-2}$                  |
| TMC-84 | $[\text{Os}(\text{NS})\text{(SeCN})_5]^{-2}$                 |
| TMC-85 | $[\text{Ru}(\text{NS})\text{(N}_3)_5]^{-2}$                  |
| TMC-86 | $[\text{Mo}(\text{NO})_2(\text{CN})_4]^{-2}$                 |

Most preferred is  $[\text{Os}(\text{NO})\text{Cl}_5]^{-2}$ . During its application, it is preferably associated with a cation, namely  $2\text{Cs}^{+1}$ , to form  $\text{Cs}_2\text{Os}(\text{NO})\text{Cl}_5$ .

If the silver halide grains of the present invention are modified by a dopant, it is preferable that the dopant be incorporated into a 93 percent core region of each silver halide grain; i.e. it is added during precipitation until 93 percent of the grain volume is formed. It may also, however, be added to the emulsion at a later stage of precipitation, as long as it is positioned below the surface of the silver halide grain.

If the silver halide grains of the present invention are modified by a grain surface modifier, it is preferable to deposit the modifier at intervals along the surface of the silver halide grains in a silver bromide carrier. The silver bromide carrier, in such instances, accounts for less than about 2 molar percent, and preferably less than about 1 molar percent, of the crystals' total halide content.

Optimally, the silver bromide carrier is a Lippmann bromide emulsion, which is a very fine grain silver bromide emulsion having average grain sizes about 0.05 microns. Such an emulsion will have incorporated in its grains certain levels of the grain surface modifier. These emulsions are digested in the presence of the much larger silver halide grains of the present invention. They are then allowed to recrystallize on the surface of the larger grains, thus delivering the grain surface modifier.

Because the Lippmann bromide carriers account for less than about 2 molar percent (and preferably less than about 1 molar percent) of the total halide in the silver halide grains, they do not form a shell around the larger grains. Rather, they form deposits at intervals along the surface of the grains. Generally, these deposits will form at the corners of the silver halide grains.

It is also possible to form the emulsions of the present invention by adding the grain surface modifier alone to a post-precipitation emulsion, or with a solution of potassium bromide.

The dopant or grain surface modifier used in the present invention is preferably applied to a silver chloride emulsion which has been ripened in the presence of a ripening agent. Also, it is preferred that they are added to the emulsion in amounts between about 0.01 and about 10 micrograms per mole of silver halide; more preferred if they are added in amounts between about 0.1 and about 5.0 micrograms per mole of silver halide; and most preferred if they are added in amounts between about 0.75 and about 2.0 micrograms per mole of silver halide.

The invention may be practiced with any of the known techniques for emulsion preparation. Such techniques include those which are normally utilized, for instance single jet or double jet precipitation; or they may include forming a silver halide emulsion by the nucleation of silver halide grains in a separate mixer or first container with later growth in a second container. All of these techniques are referenced in the patents discussed in *Research Disclosure*, December 1989, 308119, Sections I-IV at pages 993-1000.

After precipitation of the silver halide grains, the emulsions are washed to remove excess salt. They can then chemically or spectrally sensitized in any conventional manner as disclosed in the above-referenced *Research Disclosure* 308119.

Specific sensitizing dyes which can be used in accordance with the invention include the polymethine dye class, which further includes the cyanines, merocyanines, complex cyanines and merocyanines (i.e. tri-, tetra- and polynuclear cyanines and merocyanines), oxonols, hemioxonols, styryls, merostyryls, and strep-

tocyanines. Other dyes which can be used are disclosed in *Research Disclosure* 308119.

Chemical sensitizers which can be used in accordance with the invention include the gold and sulfur class sensitizers, or the transition metal sensitizers as discussed above. Further, they can be combined with known antifoggants or stabilizers such as those disclosed in *Research Disclosure* 308119, Section VI. These may include halide ions, chloropalladates, and chloropalladites. Moreover, they may include quaternary ammonium salts, tellurazolum salts, and water soluble inorganic salts of transition metals such as magnesium, calcium, cadmium, cobalt, manganese, and zinc.

After sensitizing, the emulsions can be combined with any suitable coupler (whether two or four equivalent) and/or coupler dispersants to make the desired color film or print photographic materials; or they can be used in black-and-white photographic films and print material. Couplers which can be used in accordance with the invention are described in *Research Disclosure* Vol. 176, 1978, Section 17643 VIII and *Research Disclosure* 308119 Section VII, the entire disclosures of which are incorporated by reference.

The emulsions of the invention are preferably negative working, but may also be positive-working. They are incorporated into a photographic element, and processed, upon exposure, by any known method (such as those methods disclosed in U.S. Pat. No. 3,822,129 and *Research Disclosure* 308119 Section XIX). Typically, a color photographic element comprises a support, which can contain film or paper, sized by any known sizing method, and at least three different color forming emulsion layers. The element also typically contains additional layers, such as filter layers, interlayers, overcoat layers, subbing layers, and the like. It may contain brighteners, antistain agents, hardeners, plasticizers and lubricants, as well as matting agents and development modifiers. Specific examples of each of these, and their manners of application, are disclosed in the above-referenced *Research Disclosure* 308119, and *Research Disclosure* 17643 (both incorporated by reference).

As described, the present invention also relates to a method of improving the sensitivity and stability of a silver halide emulsion. Such method comprises adding to the emulsion a photographically effective amount of an organic compound having a thiosulfonic acid substituent, an organic compound having a sulfinic acid substituent, and an amine borane. In a preferred embodiment, the method also comprises the further step of adding a photographically effective amount of a transition metal complex to the emulsion.

By photographically effective amount, it is meant an amount necessary to achieve some desired photographic effect. Such an amount is exemplified above in the description of the present invention's preferred photographic elements.

The invention can be better appreciated by reference to the following specific examples. They are intended to be illustrative and not exhaustive of the emulsions of the present invention and their methods of formation and use.

## EXAMPLES

### Preparation of emulsions

Solutions utilized for emulsion preparation:

-continued

|                      |                 |
|----------------------|-----------------|
| Gelatin              | 21.0 g          |
| 1,8-dithiooctanediol | 128.0 mg        |
| distilled water      | 502.0 ml        |
| <u>Solution B</u>    |                 |
| Silver Nitrate       | 170.0 g         |
| Mercuric Chloride    | 0.085 mg        |
| distilled water      | 327.6 ml        |
| <u>Solution C</u>    |                 |
| Sodium Chloride      | 58.0 g          |
| distilled water      | 338.3 ml        |
| <u>Solution D</u>    |                 |
| Sodium Chloride      | 53.9 g          |
| $C_2Os(NO)Cl_5$      | 0.75 micrograms |
| distilled water      | 314.6 ml        |

### Preparation of Examples 1-4

Example 1 was produced by placing solution A in a reaction vessel and stirring it at 46° C. Solutions B and C were added simultaneously at constant flow rates for 60 minutes while controlling the silver potential at 1.5 pCl. The emulsion was then washed to remove excess salts. It was heated to 40° C., after which 7.5 milligrams of gold sensitizing compound were added as disclosed in U.S. Pat. No. 2,642,361. The emulsion was then digested at 60° C. and 280 milligrams of yellow dye, 104 milligrams of 1-(3-acetamidophenyl)-5-mercaptopotetrazole, and 1033 milligrams of potassium bromide were added. The emulsion was coated on a paper support at 280 mg/m<sup>2</sup> silver along with 1076 mg/m<sup>2</sup> silver of yellow forming coupler alpha-(4-(4-benzoyloxyphenyl-sulfonyl)phenoxy)-alpha(pivalyl)-2-chloro-5-(gamma-(2,4-di-5-amylphenoxy)butyramido)acetanilide). A 1076 mg/m<sup>2</sup> gel overcoat was applied as a protective layer along with a vinylsulfone hardener. The coating was exposed for 0.1 second with a Wratten ® (trademark of Eastman Kodak Company) 2C filter through a step tablet and processed at 35° C. as follows:

|                                                                                                                                                                                |         |
|--------------------------------------------------------------------------------------------------------------------------------------------------------------------------------|---------|
| color development                                                                                                                                                              | 45 sec  |
| Bleach-fix (FeEDTA)                                                                                                                                                            | 45 sec  |
| Wash                                                                                                                                                                           | 90 sec  |
| <u>Developer composition:</u>                                                                                                                                                  |         |
| Water                                                                                                                                                                          | 800 ml  |
| Triethanolamine 100%                                                                                                                                                           | 11 ml   |
| Lithium Polystyrene Sulfonate 30%                                                                                                                                              | 0.25 ml |
| Potassium Sulfite, 45%                                                                                                                                                         | 0.5 ml  |
| N,N-Diethylhydroxylamine 85%                                                                                                                                                   | 6 ml    |
| Benesulfonic acid, 5-[{4-[bis(2-hydroxyethyl)amino]-6-methoxy-1,3,5-triazin-2-yl}amino]-2-[4-[4-methoxy-6-[(2-sulfoethyl)amino]-1,3,5-triazin-2-yl]amino]-2-sulfonyl]ethenyl]- | 2.3 g   |
| Lithium Sulfate                                                                                                                                                                | 2.7 g   |
| 1-Hydroxyethyl-1,1-diphosphoric acid 60%                                                                                                                                       | 0.8 ml  |
| Potassium Chloride                                                                                                                                                             | 1.8 g   |
| Potassium Bromide                                                                                                                                                              | 0.02 g  |
| Methanesulfonamide,N-(2-((4-amino-3-methylphenyl)ethylamino)ethyl) sulfate (2:3)                                                                                               | 4.55 g  |
| Potassium Carbonate                                                                                                                                                            | 23 g    |
| Water to make                                                                                                                                                                  | 1.0 ltr |
| pH                                                                                                                                                                             | 10.12   |

Example 2 was prepared as example 1 except that just prior to coating the emulsion on a support, 480 mg of tolylthiosulfonate(TSS) per mole of silver halide and 4800 mg of tolylsulfinate(TS) per mole of silver halide were added, the two compounds being co-dissolved in an aqueous solution.

Example 3 was prepared as example 1 except that the emulsion was treated with dimethylamine borane(D-

MAB) at a level of 0.08 mg per mole of silver halide. The samples were heated for 10 minutes at 60° C., and then coated and processed.

Example 4 was prepared as example 1 except that just prior to coating the emulsion on a support, 480 mg of tolylthiosulfonate per mole of silver halide and 4800 mg of tolylsulfinate salt per mole of silver halide were added, the two compounds being co-dissolved in an aqueous solution. Also, the emulsion was treated with dimethylamine borane at a level of 0.08 mg per mole of silver halide. The samples were heated for 10 minutes at 60° C., and then coated and processed.

All of the above emulsion precipitations had grains which were cubic and had an edge length of 0.58 microns.

The results are shown in Table 1 and correspond to sensitometric data points on each emulsions D-log E curve. Example 1 corresponds to an unmodified emulsion with neither the amine borane nor the combination of antifoggant/stabilizer compounds. As can be seen from this example, the emulsion's sensitivity is 100 and its contrast(toe) is 0.290. The emulsion also exhibits substantial instability over time as indicated by speed and toe changes of +0.16 and +0.112, respectively.

Example 2(TSS/TS only) and example 3(DMAB only) correspond to emulsions containing only one of the adjuvants utilized in accordance with the present invention. Both examples indicate improved stability. However, such stability is at the expense of a loss in sensitivity in example 2, and at the expense of a significant loss of contrast in example 3 (a softening of the toe from 0.290 to 0.346).

The invention, which is demonstrated in example 4, resides in an emulsion which exhibits increased sensitivity and excellent stability. The emulsion exhibits such characteristics with only a slight loss in contrast, a quality which was not expected given the contrast degradation caused by the reduction sensitizer (example 3) and the ineffectual nature of the antifoggant/stabilizer (example 2) on toe sharpness.

then washed to remove excess salts, and then coated and processed as above.

Example 6 was prepared and processed as example 5 except that just prior to coating the emulsion on a support, 480 mg of tolylthiosulfonate(TSS) per mole of silver halide and 4800 mg of tolylsulfinate(TS) per mole of silver halide were added, the two compounds being co-dissolved in an aqueous solution.

Example 7 was prepared as example 5 except that the emulsion was treated with dimethylamine borane(D-MAB) at a level of 0.08 mg per mole of silver halide. The samples were heated for 10 minutes at 60° C., and then coated and processed.

Example 8 was prepared as example 5 except that just prior to coating the emulsion on a support, 480 mg of tolylthiosulfonate per mole of silver halide and 4800 mg of tolylsulfinate salt per mole of silver halide were added, the two compounds being co-dissolved in an aqueous solution. Also, the emulsion was treated with dimethylamine borane at a level of 0.08 mg per mole of silver halide. The samples were heated for 10 minutes at 60° C., and then coated and processed.

Example 9 was prepared and processed in a manner similar to example 5 except that the amount of  $Cs_2Os(-NO)Cl_5$  was increased to 1.25 micrograms.

Example 10 was prepared and processed as example 6 except that example 9 was used instead of example 5.

Example 11 was prepared and processed as example 7 except that example 9 was used instead of example 5.

Example 12 was prepared and processed as example 8 except that example 9 was used instead of example 5.

Example 13 was prepared and processed in a manner similar to example 5 except that the amount of  $Cs_2Os(-NO)Cl_5$  was increased to 2.0 micrograms.

Example 14 was prepared and processed as example 6 except that example 13 was used instead of example 5.

Example 15 was prepared and processed as example 7 except that example 13 was used instead of example 5.

Example 16 was prepared and processed as example 8 except that example 13 was used instead of example 5.

TABLE 1

| Ex          | Os(NO) <sup>1</sup> | TSS/TS | DMAB | Speed <sup>2</sup> | Toe <sup>3</sup> | Speed Change <sup>4</sup> | Keeping ability Dmin Change <sup>5</sup> | Toe Change <sup>6</sup> |
|-------------|---------------------|--------|------|--------------------|------------------|---------------------------|------------------------------------------|-------------------------|
| 1 control   | 0                   | N      | N    | 100                | .290             | +0.16                     | 0.094                                    | +0.112                  |
| 2 control   | 0                   | Y      | N    | 93                 | .287             | +0.04                     | 0.044                                    | +0.087                  |
| 3 control   | 0                   | N      | Y    | 178                | .346             | +0.00                     | 0.291                                    | +0.209                  |
| 4 invention | 0                   | Y      | Y    | 141                | .316             | -0.04                     | 0.083                                    | +0.095                  |

<sup>1</sup>Micrograms of  $Cs_2Os(NO)Cl_5$ /mole of silver halide

<sup>2</sup>The reciprocal of the relative amount of light in LogE  $\times 100$  to produce 1.0 density

<sup>3</sup>The density value of the point 0.3 LogE fast of the speed point

<sup>4</sup>The change in LogE speed due to two week incubation at 100° F. and 50% humidity

<sup>5</sup>Change in minimum density at 100° F. and 50% humidity

<sup>6</sup>The change in toe density due to two week incubation at 100° F. and 50% humidity

### Preparation of Examples 5-16

Example 5 was produced by placing solution A in a reaction vessel and stirring it at 46° C. Solutions B and D were added simultaneously at constant flow rates until 93 percent of the grain volume had formed. The silver potential was controlled at 1.5 pCl. After 93% of the grain volume was formed, solution C was used in place of solution D for the remainder of the reaction, keeping the same flow rates. The total precipitation time for the emulsion was 60 minutes. The emulsion was

All of the above emulsion precipitations had grains which were cubic and had an edge length of 0.58 microns.

The results are shown in Table 2 and correspond to sensitometric data points on each emulsions D-log E curve. The data illustrates the advantageous effects of the antifoggants/stabilizers and the reduction sensitizer are found in emulsions doped with a transition metal complex containing a nitrosyl or thionitrosyl ligand.

TABLE 2

| Ex        | Os(NO) <sup>1</sup> | TSS/TS | DMAB | Speed <sup>2</sup> | Toe <sup>3</sup> | Keeping ability Speed Change <sup>4</sup> | Dmin Change <sup>5</sup> | Toe Change <sup>6</sup> |
|-----------|---------------------|--------|------|--------------------|------------------|-------------------------------------------|--------------------------|-------------------------|
| 5 control | .75                 | N      | N    | 95                 | .265             | +0.18                                     | 0.082                    | +0.126                  |
| 6 control | .75                 | Y      | N    | 93                 | .260             | +0.07                                     | 0.044                    | +0.096                  |

TABLE 2-continued

| Ex           | Os(NO) <sup>1</sup> | TSS/TS | DMAB | Speed <sup>2</sup> | Toe <sup>3</sup> | Keeping ability<br>Speed Change <sup>4</sup> | Dmin Change <sup>5</sup> | Toe Change <sup>6</sup> |
|--------------|---------------------|--------|------|--------------------|------------------|----------------------------------------------|--------------------------|-------------------------|
| 7 control    | .75                 | N      | Y    | 174                | .318             | +0.03                                        | 0.257                    | +0.215                  |
| 8 invention  | .75                 | Y      | Y    | 138                | .293             | -0.01                                        | 0.073                    | +0.109                  |
| 9 control    | 1.25                | N      | N    | 78                 | .230             | +0.23                                        | 0.061                    | +0.149                  |
| 10 control   | 1.25                | Y      | N    | 74                 | .222             | +0.12                                        | 0.031                    | +0.117                  |
| 11 control   | 1.25                | N      | Y    | 144                | .284             | +0.07                                        | 0.233                    | +0.244                  |
| 12 invention | 1.25                | Y      | Y    | 110                | .249             | +0.05                                        | 0.055                    | +0.141                  |
| 13 control   | 2.0                 | N      | N    | 74                 | .210             | +0.29                                        | 0.075                    | +0.195                  |
| 14 control   | 2.0                 | Y      | N    | 68                 | .207             | +0.15                                        | 0.033                    | +0.132                  |
| 15 control   | 2.0                 | N      | Y    | 129                | .267             | +0.14                                        | 0.256                    | +0.275                  |
| 16 invention | 2.0                 | Y      | Y    | 93                 | .234             | +0.13                                        | 0.071                    | +0.166                  |

<sup>1</sup>Micrograms of Cs<sub>2</sub>Os(NO)Cl<sub>5</sub>/mole of silver halide<sup>2</sup>The reciprocal of the relative amount of light in LogE × 100 to produce 1.0 density<sup>3</sup>The density value of the point 0.3 LogE fast of the speed point<sup>4</sup>The change in LogE speed due to two week incubation at 100° F. and 50% humidity<sup>5</sup>Change in minimum density at 100° F. and 50% humidity<sup>6</sup>The change in toe density due to two week incubation at 100° F. and 50% humidity

The invention has been described in detail with particular reference to preferred embodiments thereof but 20 it will be understood that variation and modifications can be effected within the spirit and scope of the invention.

What is claimed is:

1. A negative working photographic element comprising a support having thereon a silver halide emulsion layer, wherein said emulsion layer contains an amine borane, a thiosulfonate compound that satisfies the formula:



where

R<sup>1</sup> represents an aliphatic, carbocyclic, or heterocyclic group, which may be substituted or unsubstituted, and

M<sup>1</sup> represents any mono-, di-, or tri-valent cation; and a sulfinate compound that satisfies the formula:



where

R<sup>2</sup> represents an aliphatic, carbocyclic, or heterocyclic group, which may be substituted or unsubstituted, and

M<sup>2</sup> represents a mono-, di-, or tri-valent cation.

2. A negative working photographic element according to claim 1, wherein said emulsion layer is comprised of silver halide grains which are predominantly silver chloride.

3. A negative working photographic element according to claim 2, wherein said silver halide grains contain at least 70 molar percent silver chloride and less than 2 molar percent silver iodide, with the remaining silver halide being silver bromide.

4. A negative working photographic element according to claim 3, wherein said silver halide grains contain at least 98 molar percent silver chloride, with the remaining silver halide being silver bromide and silver iodide.

5. A negative working photographic element according to claim 4, wherein chloride is the sole halide in said silver halide grains.

6. A negative working photographic element according to claim 2 wherein the thiosulfonate compound is in an amount between about 20 and about 2300 milligrams per mole of silver halide, and the sulfinate compound is in an amount between about 10 and about 20,000 milligrams per mole of silver halide, with the ratio of the

thiosulfonate compound to the sulfinate compound being between about 20:1 and about 1:20 by weight.

7. A negative working photographic element according to claim 6 wherein the thiosulfonate compound is in an amount between about 100 and about 1500 milligrams per mole of silver halide, and the sulfinate compound is in an amount between about 100 and about 15,000 milligrams per mole of silver halide, with the ratio of the thiosulfonate compound to the sulfinate compound being between about 10:1 and about 1:10 by weight.

8. A negative working photographic element according to claim 7 wherein the thiosulfonate compound is a tolylthiosulfonate salt, and the sulfinate compound is a tolylsulfonate salt.

9. A negative working photographic element according to claim 8 wherein the amine borane satisfies the formula:



wherein

R<sup>3</sup>, R<sup>4</sup>, and R<sup>5</sup> represent hydrogen atoms, aliphatic, carbocyclic, or heterocyclic groups, which may be substituted or unsubstituted.

10. A negative working photographic element according to claim 9 comprising the amine borane in an amount between about 0.001 and about 1.0 milligram per mole of silver halide.

11. A negative working photographic element according to claim 10 comprising the amine borane in an amount between about 0.02 and about 0.2 milligram per mole of silver halide.

12. A negative working photographic element according to claim 11, wherein the amine borane is dimethyl amine borane.

13. A negative working photographic element according to claim 12 comprising dimethyl amine borane in an amount equal to about 0.05 to about 0.1 milligram per mole of silver halide.

14. A negative working photographic element according to claim 13 further comprising a transition metal complex having the formula:



wherein

M is a transition metal selected from Groups V to X, inclusive, of the periodic table;

Z is oxygen or sulfur, and together with the nitrogen forms a nitrosyl or thionitrosyl ligand;

L represents a ligand;  
m is from 4 to 7; and  
n is zero, -1, -2, or -3.

15. A negative working photographic element according to claim 14 wherein M is osmium.

16. A negative working photographic element according to claim 15 wherein the transition metal complex is  $[\text{Os}(\text{NO})\text{Cl}_5]^{-2}$ .

17. A negative working photographic element according to claim 16 comprising  $[\text{Os}(\text{NO})\text{Cl}_5]^{-2}$  in an amount between about 0.01 microgram and about 10 micrograms per mole of silver halide.

18. A negative working photographic element comprising a support and a silver halide emulsion layer, wherein said emulsion layer contains a thiosulfonate compound that satisfies the formula:



where

$\text{R}^1$  represents an aliphatic, carbocyclic, or heterocyclic group, which may be substituted or unsubstituted, and

$\text{M}^1$  represents any mono-, di-, or tri-valent cation; a sulfinate compound that satisfies the formula:



where

$\text{R}^2$  represents an aliphatic, carbocyclic, or heterocyclic group, which may be substituted or unsubstituted, and

$\text{M}^2$  represents a mono-, di-, or tri-valent cation; and an amine borane; and wherein said emulsion layer is comprised of silver halide grains which are predominantly silver chloride, and which internally contain a dopant comprised of a nitrosyl or thionitrosyl ligand

and a transition metal chosen from Groups V to X, inclusive, of the periodic table.

19. A method of improving the sensitivity and stability of a negative working silver halide emulsion comprising adding to said emulsion a photographically effective amount of an amine borane, a thiosulfonate compound that satisfies the formula:



where

$\text{R}^1$  represents an aliphatic, carbocyclic, or heterocyclic group, which may be substituted or unsubstituted, and

$\text{M}^1$  represents any mono-, di-, or tri-valent cation; and a sulfinate compound that satisfies the formula:



where

$\text{R}^2$  represents an aliphatic, carbocyclic, or heterocyclic group, which may be substituted or unsubstituted, and

$\text{M}^2$  represents a mono-, di-, or tri-valent cation.

20. A method according to claim 19 further comprising adding to said emulsion a photographically effective amount of a transition metal complex having the formula:



wherein:

M is a transition metal selected from Groups V to X, inclusive, of the period table;

Z is oxygen or sulfur, and together with the nitrogen forms a nitrosyl or thionitrosyl ligand;

L represents a ligand;

m is from 4 to 7; and

n is zero, -1, -2, or -3.

\* \* \* \* \*

40

45

50

55

60

65